

H. M. DUNN.

METHOD AND APPARATUS FOR CONCENTRATING ORE.  
APPLICATION FILED MAY 11, 1915.

1,219,089.

Patented Mar. 13, 1917.



Harry. M. Dunn.

# UNITED STATES PATENT OFFICE.

HARRY M. DUNN, OF HURLEY, NEW MEXICO.

## METHOD AND APPARATUS FOR CONCENTRATING ORE.

1,219,089.

Specification of Letters Patent. Patented Mar. 13, 1917.

Application filed May 11, 1915. Serial No. 27,348.

To all whom it may concern:

Be it known that I, HARRY M. DUNN, a citizen of the United States, and a resident of Hurley, in the county of Grant, in the 5 State of New Mexico, have invented new and useful Improvements in Methods and Apparatus for Concentrating Ore, of which the following is such a full, clear, and concise disclosure as will enable others skilled 10 in the art to which this invention relates to make and use the same.

My invention relates to the concentration of ore and particularly to that type of concentration commonly known as ore flotation.

15 It is now well known that if finely divided ore is mixed with water to form a pulp and oil, tar or grease is added to this mixture and it is agitated so that air is thoroughly mixed through the complete mixture and 20 comes in contact with the ore particles the oil, tar or grease assists the metalliferous particles of the ore to hold to them some of the air and the metalliferous particles are floated to the surface of the mixture while 25 the particles of the gangue do not hold any of the air to them and they sink to the bottom and are separated. The metalliferous particles are brought to the surface in a froth and the oil is later separated from 30 them in many well known ways. While air is the gas generally used for flotation of metalliferous particles of ore any gas may be used and this gas may be applied to the mixture either by mechanically mixing it 35 with the pulp or it may be formed in the mixture by making it acid and generating the gas by a chemical reaction.

One object of my invention is to provide 40 a process for bringing gas into intimate contact with finely divided ore, preferably in the presence of oil, tar or grease, any of which will hereinafter be termed oil, when the ore is mixed with or held in suspension in water. To this end I set in motion a 45 mixture of water and finely divided ore, said mixture preferably including a relatively small quantity of oil, by subjecting said mixture to the action of a jet of gas, then using the energy thus imparted to the mixture 50 to elevate the mixture, and then permitting it to fall back upon itself or another portion of the mixture whereby the mixture is agitated and the air is brought into contact with the particles of the metalliferous 55 constituents of the ore and adhering to them it carries them to the surface.

Another object of my invention is to provide an apparatus for bringing gas into intimate contact with particles of finely divided ore preferably in the presence of oil, when the finely divided ore is mixed with or held in suspension in water. To this end I provide means for projecting a mixture of finely divided ore and water, said mixture preferably including a small percentage of oil, 60 against a throwback plate, said plate being preferably inclosed in a chamber, whereby said mixture falls back upon itself preferably to be thrown again against the throwback plate whereby a rolling motion is imparted 65 to the mixture. The means for projecting the mixture against the throwback plate is preferably a gas operated injector. Gas is thus introduced into the mixture and the rolling motion thereof brings it into intimate contact with the oil-coated metalliferous particles of the ore. The metalliferous particles thus hold air to them and they are floated to the surface as a froth. 70

In addition to a device for bringing the 80 gas into contact with the particles of the ore, said particles preferably being treated with oil, I provide a chamber or spitzkasten in which the mixture is brought to rest in order that the gas may bring the particles 85 of the metalliferous constituents to the surface of the mixture as a froth and also a receptacle or launder into which the froth is deposited preparatory to freeing it of oil. 90

In the device hereinafter described as embodying my invention and carrying out my process the mixture is projected into the chamber containing the throwback plate and against said plate by an air operated injector which draws the mixture into it from 95 the lower part of the chamber or spitzkasten and as the mixture passes through the injector oil is fed to it. I do not, however, intend that my invention shall be limited to this means of projecting the mixture against 100 the throwback plate, nor that it shall be limited to the use of a throwback plate as means for causing the mixture to fall back upon itself to agitate it, for I intend that my invention shall be defined by the here- 105 unto appended claims.

Other and further advantages and objects will appear from the following description taken in connection with the accompanying drawings forming a part of this specification and be pointed out in the claims. 110

In the accompanying drawings in which

like reference characters indicate like parts. Figure 1 is a view of a series of cells, partly broken away, which embody my invention; Fig. 2 is a perspective sectional view taken on the line 2—2 of Fig. 1; Fig. 3 is a sectional detail view of the oil spraying nozzle; and Fig. 4 is a sectional view of a modified form of a gas injector.

In concentrating ore according to the process embodying my invention the ore is finely divided and mixed with water which holds it in suspension forming what is commonly known as pulp. This pulp is fed from a mixer by a trough 1 into a tank 2 which converges toward its bottom and in which the pulp thickens. It is fed through a spigot 3 into a riser 4 of a feed conduit 5 from which it passes through the opening 6 into the spitzkasten or chamber A of the first cell 7. The succeeding cells 8 and 9 are similar to the cell 7, each having a chamber A and the treatment of the pulp while in each chamber will later be stated in connection with a description of a single cell.

The chamber A of each cell communicates with the chamber A of each succeeding cell through an opening 10 and the last cell opens into a tailings trough 11 through a similar opening 10. The flow through the openings 10 is impeded by a partition 12 in each cell, and the flow through the opening 6 and the openings 10 is restricted so as to preserve a correct level of liquid in each cell by a gate 13 operated in any well known manner by a hand-wheel 14.

Adjacent to each chamber or spitzkasten A is a mixing or agitating chamber B separated from chamber A by a wall 15. Through this wall 15 extends one leg 17' of each of two substantially L-shaped pipe sections 17, the other leg 17" of which extends toward the bottom of chamber A. Through the wall of each pipe section 17 extends a gas pipe 16 positioned axially of the leg 17' and extending across the opening whereby the leg 17" communicates with the leg 17'.

Oil, grease or tar is fed through a pipe 18, preferably under pressure, whereby it is atomized by the nozzle 19, but in the modification shown in Fig. 4 it need not be under great pressure as the oil which is supplied through the usual pipe 16 is conducted in through the side of the leg 17" of the pipe section 17 by means of the pipe-end 119 so that it is fed directly into the pulp as it enters the leg 17".

Pulp enters one side of the chamber or spitzkasten A and as gas is forced in to the gas pipe 16 it receives a charge of oil in the form of a spray from the nozzle 19, and as the air so charged passes out of leg 17' pulp is carried in to the leg 17" by the entraining action of the air. The pulp is thus preliminary mixed with the gas and oil and it has imparted to it a considerable

velocity by the action of the gas. It is projected substantially horizontally against the vertically curved throwback plate 20 whereby it is elevated and falls back upon itself. As the chamber B fills up there is a stream of the complete mixture rising along the surface of the plate 20, and the stream from the leg 17' entrains some of the mixture and carries it into the rising stream so that there is a downward flow along the wall 15 and the whole mass has a rolling motion as indicated by the arrows  $\alpha$ ,  $\alpha$ . This rolling motion is thus due to a rising of one portion of the mass and permitting the rising part to fall back upon itself and upon the remainder of the mass and an entraining of a part of the otherwise stationary mass and I have found this rolling motion extremely efficient in bringing the gas into intimate contact with the oil-coated particles of the metalliferous constituents of the ore.

As the level of the mixture rises in the chamber B the larger bubbles will throw the lighter froth which forms over the wall 15 and it will pass down between the wall 15 and the curtain 21 onto the top of the mass of pulp in the chamber A which rises approximately to the level of the lower edge of the curtain 21 to form a seal, at least when the froth forms on the top of the pulp. The level of the froth continues to rise as the mixer operates and the froth is drawn off over the lip K into the launder L which extends across the front of each cell. The launders discharge into one another as indicated in Fig. 1 and then into the ore bin 22 in which the froth is collected and the oil is later separated from the metalliferous particles.

It will be seen that the pulp is fed into the bottom of each chamber A and retarded from passing out therefrom by the partition 12 until it has been projected into the chamber B so that it is the pulp which has been thrown over the top of the wall 15 which passes over the top of the partition 12 and into the next chamber A of the next cell. It will be seen, therefore, that what particles of the metalliferous constituents of the ore are not floated in one cell will be acted on in the next cell and floated therein. It will be seen from the structure thus described that the pulp enters the first cell through the opening 6. It is then ejected from the chamber A by the gas operated injectors into the chamber B against the throwback plate. After being thoroughly agitated as described it is thrown over the wall 15 onto the top of the pulp in the chamber A, and it then flows over the top of the partition 12 through the opening 10 into the chamber A of the next cell. The pulp which enters a chamber A is prevented from flowing out therefrom until it has been agitated in the chamber B of the same cell by the partition 130.

12 in the given chamber A. Whatever froth forms in any chamber A is drawn over the lip K into the launder L of that cell and flows through the launders L of the other 5 cells into the bin 22.

In the top of each chamber B there are 10 vent pipes 23 to let the gas out which bubbles up through the pulp therein so that the seal formed by the curtain 21 will not be broken.

While I have described a specific embodiment of my invention with great detail I do not intend that my invention shall be limited to the features herein disclosed but 15 intend that modifications thereof may be made which occur to those skilled in the art and that my invention shall be defined by the hereunto appended claims only.

What I claim and desire to secure by Letters Patent of the United States is the following:

1. The herein described method of concentrating ores which consists in imparting an upward velocity in substantially vertical 25 planes only to a stream of a mixture of pulp and a frothing agent, permitting the elevated portion of the stream to fall back upon itself in contact with a free atmosphere whereby air is entrained in the mixture, and separating the froth produced 30 thereby.

2. The herein described method of concentrating ores which consists in adding a frothing agent to a stream of pulp, discharging 35 gas into the stream to impart a velocity thereto, discharging said stream upwardly in substantially vertical planes only, permitting said stream to fall back upon itself in contact with a free atmosphere whereby 40 additional air is entrained and the whole mass is agitated, and separating the froth produced thereby.

3. The herein described method of concentrating ores which consists in forcibly 45 impelling a stream of a mixture of a frothing agent and pulp to rise through and in contact with a body of such a mixture to a point above the said body, permitting a portion of the part of the mixture so elevated 50 above the body to fall back thereupon in contact with a free atmosphere forming a froth and separating the froth.

4. The herein described method of concentrating ores which consists in imparting a 55 velocity to a portion of a body of a mixture of pulp and oil, permitting said portion to flow through and in contact with the remainder of the body, deflecting the moving portion upward so that it rises above the 60 remainder of the body and permitting it to fall back upon itself forming a froth.

5. The herein described method of concentrating ores which consists in imparting

a velocity to a portion of a body of a mixture of pulp and oil, permitting said portion 65 to flow through and in contact with the remainder of the body, deflecting said moving portion upward so that it rises above the remainder of the body and permitting it to fall in contact with a free atmosphere back 70 upon the remainder of the body forming a froth.

6. The herein described method of concentrating ores which consists in adding oil to a stream of pulp and discharging gas into 75 the stream to impart a velocity thereto, projecting the resulting stream of said mixture into the body of a similar mixture, elevating a portion of said body by the energy of said stream and permitting said elevated portion 80 to fall in contact with a free atmosphere back upon said body from a point above the body forming a froth.

7. In an apparatus for concentrating ores, a chamber, a wall dividing said chamber into 85 compartments, one of said compartments having a vertically curved wall, a gas operated injector extending through said dividing wall for discharging the contents of one compartment into the other and against 90 said curved wall.

8. In an apparatus for concentrating ores, a compartment having a vertically curved wall, a gas operated injector for projecting 95 a mixture of pulp and oil and a frothing agent into said compartment and against said wall to form a froth, and means for separating the froth formed thereby.

9. In an apparatus for concentrating ores, a chamber, a wall extending from the bottom 100 to a point near the top thereof and dividing it into compartments, a gas operated injector extending through said wall for discharging the contents of one compartment into the second compartment and a vertically 105 curved throwback plate in said second compartment against which the contents of the first compartment is discharged.

10. In an apparatus for concentrating ores, a chamber, a wall extending from the bottom 110 to a point near the top thereof and dividing it into compartments, a gas operated injector for discharging the contents of one compartment into the second compartment, a curtain wall extending from the 115 top of the first compartment to a point below the top of said wall and a vertically curved throwback plate in said second compartment against which the contents of the first compartment is discharged.

In testimony whereof, I have hereunto set my signature this 16th day of April, 1915.

HARRY M. DUNN.

Witnesses:

C. W. McSHERRY,  
T. C. McSHERRY.